# EUROPEAN PATENT APPLICATION

(11) **EP 0 805 131 A1**
(43) Date of publication of application: **05.11.1997**
(21) Application number: 95937890.2
(22) Date of filing: 17.11.1995
(51) Int. Cl.: C06F 3/08, C06B 39/00

(54) **PAINTS FOR SERIGRAPHIC APPLICATION OR THE LIKE, INTENDED TO GENERATE FRICTION SURFACES FOR MATCHES, AND PRODUCTION PROCESSES**

(71) Applicant: Sericyt S.a.L., 28960 Humanes de Madrid (ES)
(72) Inventor: CALVO SAN PEDRO, Antonio, E-28960 Humanes de Madrid (ES)
(74) Representative: Perez Bonal, Bernardo
(86) International application number: ES9500128
(87) International publication number: WO9719037

(57) **Abstract**

They comprise phosphorus activated or not by a metal compound bringing oxygen to the combustion, and an acrylic varnish which, together with a vinyl polyacetate, may be used as keying agent and binders with respect to consistent substrates or charges, with minimum cost and layer thickness, in a plurality of shapes and colours, with a composition appropriate to a wide range of natural materials, laminates or plastic coats therefor, with the fluidity and drying velocity appropriate for printing, the most complex preparation being obtained by beating part of the varnish and, when appropriate, the vinyl polyacetate together with the phosphorus, homogenizing the mixture, milling together with the quartz and mixing with another milled mixture of the rest of the varnish together with the metal oxide.

## Description

### OBJECT OF THE INVENTION

The invention proposed herein consists in serigraph or similarly applied paints for generating match friction surfaces and in the procedures for the obtainment thereof, said paints (preferably comprising serigraph ink, although silkscreen applications and other applications are not discarded) consisting in a basic pigment, preferably red phosphorus, which is an inflammable product activated or not by a metal compound contributing oxygen to the combustion and which is mixed with a polymer, namely an acrylic varnish, which may or may not act as an adhesiveness or binding agent for solid substrates or fillers which moreover increase the phosphorus friction surface while serving to curb the spreading of the combustion onto the rest of the scraper resulting from the final serigraph or similar printing.

These paints, of a minimum cost and layer thickness, are presented in multiple shapes and colours and in compounds applicable to a wide range of natural materials, as well as plastic sheets and covers for said materials, in certain cases incorporating additional agents which enhance ink adhesiveness; other cases, involving exceedingly stable materials, must be surface pre-treated.

The more simple serigraph ink, silkscreen or similar preparation procedure consists in the simple stirring of acrylic varnish and phosphorus, and the most complex among those proposed consists in stirring the main portion of the acrylic resin and its appropriate solvents (acetates, acetones, aromatic solvents and mixtures thereof), plus vinyl polyacetate to which phosphorus is added to achieve a homogeneous mixture which is ground after incorporating conventional filler materials such as quartz and carbonates. For safety reasons, the remaining resin solution is mixed separately with the conventional metal oxide, and is then ground.

Following the joint mixture and homogenization, a product is obtained which has a much lower phosphorus content than that of the normal scrapers, with a fluency and drying speed suitable for conventional serigraph, silkscreen, etc. application, as in the case of any standard ink.

### BACKGROUND OF THE INVENTION

The traditional formula for match box and match folder scrapers in the form of a continuous band extended by rollers offers no alternative application, with the additional drawback that it is difficult to apply by techniques differing from that of band laminating.

The conventional formula incorporates a resin, usually in the form of a vinyl polyacetate copolymer and polyethylene, although it can also comprise only polyacetate, water and pure ammonia as a stabilizer in a resulting amount in the order of 19% by weight; quartz or carbonate in a similar 17% by weight proportion, in which the zinc oxide seldom exceeds one tenth, and, finally, phosphorus in the amount of 64% by weight.

On the other hand, the cost of phosphorus, even red phosphorus, is very high in comparison with the cost of resin - namely three or four times as high - so that the reduction in the price of the basic pigment is substantial, considering its percentage in the formula.

However, this high phosphorus content originates from the natural aggregation of a number of pigments in the form of glomerules which, by virtue of this aggregation, offer a reduced enveloping surface considerably inferior to that of the set of individual pigments, thereby proportionately reducing its inflammation capability and increasing the need for phosphorus inclusion.

Since water-based adhesives are involved, no grinding is possible, either together with or separated from the fillers, and the phosphorus from the fillers, so that glomerule reduction or disintegration, and thus proportionate reduction of the phosphorus content, is impossible.

On the other hand, the pasty mass from which the scraper band derives clogs the serigraphy screen and thus obstructs subsequent steps in the procedure. Resorting to a higher dilution is of no avail, and additional problems are bound to be encountered deriving from the thickness of the band being laminated as a result of pigment agglomeration, apart from the fact that an excess of liquid would impair the band's geometrical rectangular-section shape from being formed, which would protrude over the band edges.

In any event, the traditional formula is inadequate for depositing over plastics in general, and very particularly over specific films such as the cellulose diacetate films normally used in cardboard plasticizing.

Finally, despite the fact that earlier examples exist wherein match box scrapers are provided in multiple colours - red, yellow, white, mauve, blue, etc. - beyond the colours of the commercially available phosphorus varieties, their exclusive application as a roller-laminated band dismisses any earlier connection with the present invention.

The same applies to the grinding procedures designed to produce red phosphorous from yellow phosphorus, its application differing totally from the present invention, as will become apparent hereinafter.

### DESCRIPTION OF THE INVENTION

The invention that is the object of the present specification, comprising serigraph, silk screen or similarly applied paints for the printing of variously shaped surfaces with a very thin layer for the lighting of matches by friction, and their obtainment procedure, of the type consisting in providing an inflammable pigment - e.g. red phosphorus - mixed with an adhesiveness polymer characteristic in that it is an acrylic varnish.

The resin may also bind to solid substrates for reducing pigment provision requirements and increasing the friction surface, in addition to curbing the spreading of the combustion to the rest of the scraper, and may also incorporate a metal component contributing oxygen to the combustion.

This paint is characteristic in that it is constituted by a serigraph printing ink, transferred by silkscreen or similar process, the final product having a controlled drying period that is longer than that of the conventional scraper, characteristic, for the above reason and because of its greater fluidity, in that it is ideal for fine printing operations devoid of screen or transfer means clogging problems, and which furthermore has a minimum cost and thickness, the conventional application of the scraper being achieved in multiple shapes and over a wide range of natural materials, such as paper, cardboard and plastic sheets such as PVC or plastic covers applied to said natural materials, provided said plastics or covering sheets meet the requirement of being relatively unstable, or else being applied to very stable plastics such as polyethylene and polypropylene after electrostatic, mechanical and/or chemical stripping or similar treatment of the printing surface.

In its normal version, used on paper, cardboard and certain plastics, either as a covering or as a laminar piece, such as PVC, the conventionally selected inflammable agent is red phosphorus because of its low cost and good handling functions in ink production by simply mixing it with and acrylic varnish or a solution based on solvent and plasticizer adequate for the acrylic resin which substitutes both the known polyacetate resin and the rest of the components of the laminar mass for the conventional scraper bands applied to match boxes and match folders.

The phosphorus to resin relationship is optimized in both weight and price, so that their respective 64 and 19 percentages by weight in a 3.37 quotient, practically unaltered since their invention, pass on, in the most common ink of the preferred example, to quotients which vary between 0.68 (of the greater ink fluidity) and 2.70 (of the greater consistency) with a more normal application value of 1.46 based on each circumstance resulting from a combination of endogenous and exogenous factors never before considered in conventional scrapers, ranging from the type of print-receiving material and the type of phosphorus selected for the ink to the phosphorus content in the match itself, in a range of printing possibilities for the ink which cannot be achieved by the laminate in the traditional conventional mass.

The most complex obtainment procedure among those proposed consists, generally speaking, in disintegrating the pigment aggregate in a closed grinding operation (particularly through the modern so-called pearl mills), disregarding roller grinding and thus eliminating the remote possibility of inflaming the phosphorus and practically reducing the pigment to little more that its unitary forming elements, limited by excessive ink fluidity or the defective functionality of the scraper obtained, so that the inflammable surface is proportionately increased and the phosphorus requirement is reduced accordingly, providing the above-mentioned consequent favorable economic repercussion, apart from the fact that this paint acquires the serigraph ink's normal fluidity, as opposed to the pasty laminated mass in the previous state of the art.

The solid substrate or filler, normally comprising quartz, although for different reasons, among them those relating to printing, may also be conventional carbonate deriving from at least two different types or granular sizes which is ground together with the mixture of phosphorus and varnish, while the conventional metal oxide, which is normally zinc because of cost considerations, although optionally other metal oxides may be used, such as antimony, for printing reasons such as coloring agent adjustment, for example, or for other utility reasons, such as the phosphorus content in the match, is the oxygen contributing element which enhances the phosphorus inflammability features.

The joint grinding with the pigment increases the relative surface of the filler so that its contribution may be reduced considerably, in the event of maximum phosphorus supply, or increased in order to help toward said phosphorus inflammability.

Varnish absorption by the filler is hardly taken into account because of the filler's low tixothropy, which allows for this phosphorus-filler correlation without considering the varnish as a result of the low liquid absorption capability shown by the fillers.

More specifically, the 17% by weight proportion of the filler in the traditional mixture reaches maximum values of 25% in the event that phosphorus presence is reduced to a minimum (23%), as well as minimum values of 9% by weight in the event of a maximum contribution thereof (63.5%), a mean value being established at 15.8% for a phosphorus content of 46% by weight.

In certain plastic covering applications with inadequate adhesiveness conditions, e.g. over the fine cellulose diacetate film conventionally and normally used in cardboard plasticizing because of its excellent external finish, a small proportion of simple vinyl polyacetate is incorporated to the acrylic resin in the necessary amount for providing sufficient adhesiveness to the paint or ink.

As an alternative to the acrylic resin, vinyl or other resins may be used with the corresponding complementary additions for printing on a material such as the one previously mentioned, incorporating small proportions of vinyl polyacetate and using, for example, a PVA/PVC copolymer and thus further enhancing the ink's adhesiveness.

Exceptionally, other types of phosphorus may be included, such as white or yellow phosphorus, and, depending on the printing requirements, different colours may be added to achieve the desired colour.

The printing may be of the continuous band type, although given the tendency of the match folders toward acquiring the most extravagant shapes imaginable, only limited by the application of the scraper band, greater variation is foreseen in view that printing freedom is now available for the scraper, so that any flat geometrical shape may be provided for the scraper, in any arrangement over the match folder of box.

Thus, from rectangular bands to geometrical figure arrangements either aligned or in quincunxes, as for instance a multiplicity of hexagons, in addition to irregular shapes for the scraper, in any arrangement also including letters and other graphic signs, and, when the sales promotion is launched by the tobacco manufacturers, the printed brand or corporate images are converted, for example, into the very scrapers with no practical limitation, and the same applies to the colours.

The serigraph, silkscreen or similar ink preparation procedure involves mixing the main portion of the resin, appropriately dissolved, and adding phosphorus until the mixture is homogenized and subsequently ground after incorporating the conventional material fillers, namely either quartz or carbonates.

The remaining resin solution is mixed separately with the conventional metal oxide, either zinc, antimony or other, and is then ground separately from the phosphorus for safety reasons.

Following the joint mixture and homogenization, a product is obtained which has a much lower phosphorus content than that of the normal scrapers, with a fluency and drying speed suitable for conventional serigraph, silkscreen, etc. printing, as in the case of any standard ink.

### DESCRIPTION OF THE DRAWINGS

In order to complement the description set forth and provide a better and easier understanding of the characteristics of the invention, a diagram is attached to this specification wherein the following is represented in an illustrative and non-limiting character:

The single figure shows a diagram of the procedure to be followed for obtaining the product that is the object of the most complex execution of the invention.

### PREFERRED EMBODIMENT OF THE INVENTION

As shown in said diagram, the proposed invention consists in serigraph or similarly applied paints for generating match friction surfaces, and in the procedures for the obtainment thereof, of the type consisting in providing an inflammable pigment, characterized in that they are bound to an acrylic varnish by simple mixture and, after grinding, form a serigraph printing ink for silkscreen or similar transfer providing a final product revealing a controlled and extended drying period and great fluidity and having a minimum cost and thickness, forming a scraper with a finishing that presents multiple shapes and colours applied over a wide range of natural materials such as paper and cardboard, in addition to plastic PVC sheets, or a wide range of plastic covers.

In other inks, the pigment is mixed with the acrylic varnish and a polymer such as vinyl polyacetate, and is applied to relatively unstable plastic covers such as cellulose acetates, thereby increasing their adhesiveness.

In still other inks, the resins become bonding agents applied to solid substrates or filler designed to increase the friction surface and curb the spreading of the combustion to the rest of the scraper, while reducing the pigment's contributing requirements, which pigment may be activated or not by a metal compound contributing oxygen to the combustion.

Lastly, very stable plastics such as propylene require their surface to be treated by any conventional procedure.

Variations of the general serigraph printing ink formula for silkscreen transmission, etc., are presented in the following examples:
Example 1. In the first and most representative example, applied over paper, cardboard and plastics such as PVC, or over most of the plastic covers thereof, red phosphorus and acrylic varnish are dissolved according to ink fluidity, the required solvents being incorporated to the mixture which is subsequently ground to provide the following percentages over the total weight of the mixture:

| Ink: product | Fluid % minimum | Normal % average | Thick % maximum |
|---|---|---|---|
| acrylic varnish | 59.7 | 40.7 | 27.0 |
| phosphorus | 40.3 | 59.3 | 73.0 |

Example 2. For specific applications on plastic covers with inadequate adhesiveness, such as cellulose diacetate, to the acrylic resin of the preferred example is applied a small proportion of a simple vinyl polyacetate (VPA) for a normal ink in the order of 36.2% by weight, part of the acrylic varnish being replaced by 14.5% by weight of vinyl polyacetate (VPA), the proportions thereof being adjusted to approximately 21.7% by weight, the obtainment procedure also being maintained and performing the mixture and its subsequent grinding as though only acrylic varnish were involved. The margins are as follows, in percentages over the total weight of the final resulting mixture:

| Ink: product | Fluid % minimum | Normal % average | Thick % maximum |
|---|---|---|---|
| acrylic varnish/VPA | 54.9 | 36.2 | 23.4 |
| phosphorus | 45.1 | 63.8 | 76.6 |

Example 3. This alterative paint also includes the solid substrate or filler (quartz) with two different granule sizes, namely very fine and normal, as well as a zinc metal oxide which, for a normal fluidity ink represent respective 13.2% by weight of the quartz and 2.6% by weight of the zinc incorporated as a joint percentage over the total weight of the mixture:

| Ink: product | Fluid % minimum | Normal % average | Thick % maximum |
|---|---|---|---|
| acrylic varnish/VPA | 52.0 | 38.2 | 27.5 |
| phosphorus | 23.0 | 46.0 | 63.5 |
| quartz/zinc oxide | 25.0 | 15.8 | 9.0 |

The ink (6) preparation procedure comprises stirring (I) the major portion of the varnish (2) in a conventional solution of the acrylic resin with the appropriate solvents and with the addition of VPA (1), phosphorus (3) being added to the point where the mixture is homogenized and is subsequently ground, after incorporating the quartz fillers (4), in a closed grinding machine (II), the pigment and the fillers being thoroughly disintegrated, with no limit save for the excess of fluidity of the ink obtained, while the rest of the varnish (2) is mixed (I') separately from the zinc oxide (5) and is ground (II''), both mixtures being subsequently and jointly homogenized (I'') once the adequate fluidity is achieved for conventional serigraph, silkscreen, etc. printing.
Example 4. The acrylic resin is replaced by a vinylic or other type of resin, in similar weight proportions and variations thereof, also accepting complementary additions which are identical to those of the preceding Example 2 for the above printing, either by adding small proportions of vinyl polyacetate or by using a VPA/VPC copolymer, as well as the various fillers of the preceding Example 3 being incorporated to the ink in similar weight proportions and following the same manufacturing procedure as that of said Example 3.

The scraper, printed with any of the previously mentioned inks, may be arranged in any position over the folder or box, as well as under any figure, from rectangular strips to geometrical figure arrangements, either aligned or in quincunxes or other totally irregular shapes.

This description need not be more extensive in the understanding that an expert on the subject will have sufficient information to perceive the scope of the invention and the advantages deriving therefrom, and also to reproduce said invention.

It should be understood that, provided the essence of the invention is not altered, the materials, shape, size and arrangement of the elements are liable to variation.

The terms used in this description, and their meaning, must always be taken in a non-limiting sense.

## Claims

1. Serigraph or similarly applied paints for generating match friction surfaces of the type providing an inflammable pigment, characterized in that an acrylic varnish is incorporated together with the pigment to constitute a serigraph printing ink for silkscreen or similar transfer, the resulting product having a longer and more controlled drying period, great fluidity, an adequate tixotrophy and a minimum cost and thickness under the shape of a scratcher applied to a wide range of natural materials such as paper and cardboard, as well as PVC sheets or a wide range of plastic coverings, which may be arranged in any location over the folder or box, as well as under any figure, from rectangular strips to geometrical figure arrangements, either aligned or in quincunxes or other totally irregular shapes.

2. Serigraph or similarly applied paints for generating match friction surfaces, according to the preceding claim, characterized in that the inflammable pigment is red phosphorus plus acrylic varnish in a solution which, according to the fluidity of the ink, incorporates, together with an acrylic resin, the appropriate solvents (acetates, acetones, aromatic solvents and mixtures thereof) in the following percentages over the total weight of the mixture:
| Ink: product | Fluid % minimum | Normal % average | Thick % maximum |
|---|---|---|---|
| acrylic varnish | 59.7 | 40.7 | 27.0 |
| phosphorus | 40.3 | 59.3 | 73.0 |

3. Procedure for obtaining a serigraph or similarly applied paint for generating match friction surfaces, according to the preceding claims, characterized in that, by simply stir mixing the red phosphorus and the acrylic varnish, after grinding, a serigraph printing ink of a silkscreen or similar transfer is formed.

4. Serigraph or similarly applied paints for generating match friction surfaces, according to the first claim, for specific application over plastic coverings having an inadequate adhesiveness, such as cellulose acetate, characterized in that, for a normal ink having approximately 36.2% by weight of resin, part of the acrylic varnish is replaced by 14.5% by weight of vinyl polyacetate (VPA), its proportions being adjusted to approximately 21.7% by weight in addition to establishing margins in percentages over the total weight of the final resulting mixture, namely:
| Ink: product | Fluid % minimum | Normal % average | Thick % maximum |
|---|---|---|---|
| acrylic varnish/VPA | 54.9 | 36.2 | 23.4 |
| phosphorus | 45.1 | 63.8 | 76.6 |

5. Procedure for obtaining a serigraph or similarly applied paint for generating match friction surfaces for specific application over plastic coverings having an inadequate adhesiveness, such as cellulose acetate, according to the fourth claim, characterized by simply stir mixing the red phosphorus and the acrylic varnish plus the VPA to form, after grinding, a serigraph printing ink of a silkscreen or similar transfer.

6. Serigraph or similarly applied paints for generating match friction surfaces, according to the preceding claims, which increase the friction surface and curb the spreading of the combustion to the rest of the scraper, characterized in that the acrylic resin or the acrylic resins and the VPA constitute filler binders, the pigment weight contribution requirements being reduced and the pigment being activated or not by a metal compound which contributes oxygen to the combustion.

7. Serigraph or similarly applied paints for generating match friction surfaces, according to the sixth claim, characterized in that the solid substrate or filler is quartz, in addition to zinc oxide, which, for an ink with a normal fluidity, represent respective percentages of 13.2% by weight of the quartz and 2.6% by weight of the zinc and which are incorporated in joint percentages over the total weight of the mixture, namely:
| Ink: product | Fluid % minimum | Normal % average | Thick % maximum |
|---|---|---|---|
| acrylic varnish/VPA | 52.0 | 38.2 | 27.5 |
| phosphorus | 23.0 | 46.0 | 63.5 |
| quartz/zinc oxide | 25.0 | 15.8 | 9.0 |

8. Procedure for obtaining a serigraph or similarly applied paint for generating match friction surfaces, according to the seventh claim, characterized in that it is implemented by stirring most of the varnish in a conventional solution of the acrylic resin in its appropriate solvents, with the addition of VPA, to which is added phosphorus until the mixture is homogenized, subsequently grinding it after incorporating the quarts fillers in a closed grinding machine, thoroughly disintegrating the pigment, with no limit being imposed other than the excess of fluidity of the ink to be obtained, while the rest of the varnish is mixed separately with the zinc oxide, followed by grinding, and both mixtures are subsequently jointly homogenized once the appropriate fluidity is obtained for conventional serigraph, silkscreen, etc. printing, similar to that of standard inks.

9. Serigraph or similarly applied paints for generating match friction surfaces, according to the fist to third and sixth to eighth claims, for specific application over very stable plastics such as polypropylene, characterized in that its surface is previously adequately eroded by any conventional procedure.

10. Serigraph or similarly applied paints for generating match friction surfaces, according to the fist, second, fourth, sixth, seventh and ninth claims, characterized in that the acrylic resin or the acrylic resin plus VPA are replaced by a vinylic or other type of resin in similar weight proportions and variations.

11. Serigraph or similarly applied paints for generating match friction surfaces, according to claims forth to ninth, characterized in that the acrylic resin and the vinyl polyacetate are replaced by a VPA/VPC copolymer in similar weight proportions.

12. Serigraph or similarly applied paints for generating match friction surfaces, according to claims forth to ninth, characterized in that the red phosphorus is replaced by other types of phosphorus, such as the white or yellow phosphorus, and, based on the printing colour requirements, other dyes may be added which are different to any of them.
